

# UNITED STATES PATENT OFFICE.

LEOPOLD SCHÜTZE, OF LEIPZIG-EUTRITZSCH, AND ROBERT FISCHER, OF LEIPZIG-REUDNITZ, GERMANY.

## PRINTING-COLORS.

1,096,198.

Specification of Letters Patent. Patented May 12, 1914.

No Drawing.

Application filed June 5, 1913. Serial No. 771,968.

*To all whom it may concern:*

Be it known that we, LEOPOLD SCHÜTZE, a subject of the German Emperor, and ROBERT FISCHER, a subject of the Emperor of Austria-Hungary, and residents, respectively, of Leipzig-Eutritzsche and Leipzig-Reudnitz, in the Kingdom of Saxony, German Empire, have invented new and useful Improvements in Printing-Colors, of which the following is a full, clear, and exact specification.

Our invention relates to improved printing compositions and particularly to printing colors, which are especially suitable for that mode of printing which uses engraved printing surfaces. The colors hitherto proposed for this purpose suffer from several defects. In order to obtain comparatively great fluidity, which is necessary in particular cases, the color is mixed with a diluent; the latter is volatile whereby the uniformity of the color is affected. Moreover, the color is apt to harden, the odor of the vapor of the diluent is objectionable and the vapor is injurious to health and dangerous by its inflammability. In addition to these objections the color is difficult to remove satisfactorily by the doctor, that is to say it is not completely separated by the doctor from the unengraved portions of the printing roller, so that a smudged print is produced. A still further objection is inherent in many such colors, namely that they attack the parts of the machine. By the present invention all these objections are overcome by using a special vehicle for the color. This vehicle is made by digesting albumin which has been emulsified or dissolved by addition of alkali or an alkaline salt, with a sulfonated oil or a salt thereof; for the better emulsification of the mixture there may be added a suitable medium, such as an ethereal oil. With this vehicle there may be mixed any of the colors or dyestuffs suitable for the work to be done, particularly organic dyestuffs and lakes obtained therefrom; the color or dyestuff or lake is best used in the form of a paste in order to insure satisfactory distribution in the vehicle. The manufacture of the vehicle and its mixture with the color or dyestuff may be combined into a single operation. The printing colors thus obtained, which need not contain any volatile constituent, are satisfactorily per-

manent so that the color is always uniform 55 and yields uniform printing. The colors have no objectionable odor and are not injurious to health. They are quite amenable to doctoring so that the portion of the color which has not entered the engraved lines of 60 the printing roller can be completely removed by the doctor and clear prints be obtained. Moreover, the very fine distribution of the color particles and of the vehicle renders possible an essentially finer detail 65 in the printing and the print neither runs nor bleeds. The printing rollers or plates are in no way injured or attacked by the colors. The capacity for drying exhibited by the printing colors is good and at the 70 same time they do not dry on the roller or plate when this is left at rest for a long period. The nature of the vehicle prevents the settling of the color. The printing colors go a long way in printing and are insoluble 75 in water. By suitable selection of the dye-stuffs very various tints may be obtained. Although the colors are particularly suitable for printing with engraved rollers or plates, it is obvious that by suitably varying 80 the proportions, and therefore the consistency and concentration, the colors may be used for other modes of printing.

The following are examples of how a printing color may be made according to 85 the invention.

Example 1: 125 grams of calcined sodium carbonate are dissolved in 6 liters of water and 535 grams of albumin are introduced while stirring. To this mass are added 1 90 kilo 125 grams of sodium sulfuricinoleate and the mixture is further mixed with 500 grams of refined rosin oil or turpentine oil. To the vehicle thus prepared are added 9 kilos of a paste containing 30 per cent. of 95 the precipitate formed from naphthol black and barium chlorid, and the whole is ground in a color mill. The color paste may be mixed in before the addition of sodium sulfuricinoleate.

Example 2: Instead of the solution of 125 grams of calcined sodium carbonate in 6 liters of water a solution of 85 grams of caustic potash in 5 liters of water is used. The other steps are the same as in Example 1. 105

Example 3: Instead of 9 kilos of the naphthol black paste referred to in Example 1. 9 kilos of a paste containing 30 per cent. of

the precipitate formed from naphthol black, naphthol yellow and barium chlorid is used. The other steps are the same as in Example 1 or 2.

5. Example 4: 150 grams of calcined sodium carbonate are dissolved in 5 liters of water and 500 grams of albumin are introduced while stirring. To this mass are added 1 kilo 125 grams of sodium sulfuricinoleate.
- 10 To the vehicle thus prepared 10 kilos of a paste containing 30 per cent. of the precipitate from naphthol black and barium chlorid are added, and the whole is ground in a color mill.

15 What we claim is:—

1. As a new article of manufacture, a printing composition, containing albumin, an agent for distributing same in water, water and a sulfo derivative of an oil.
- 20 2. As a new article of manufacture, a printing composition, containing albumin, an agent for distributing same in water, water, a sulfo derivative of an oil and an ethereal oil.
- 25 3. As a new article of manufacture, a printing composition, containing albumin, an agent for distributing same in water, water and a salt of a sulfonated oil.
4. As a new article of manufacture, a 30 printing composition, containing albumin, an agent for distributing same in water,

water, a salt of a sulfonated oil and an ethereal oil.

5. As a new article of manufacture, a 35 printing composition color comprising a suitable color and a vehicle containing albumin, an agent for distributing same in water, water and a sulfo derivative of an oil.

6. As a new article of manufacture, a 40 printing composition color comprising a suitable color and a vehicle containing albumin, an agent for distributing same in water, water, a sulfo derivative of an oil, and an ethereal oil.

7. As a new article of manufacture, a 45 printing composition color comprising a suitable color and a vehicle containing albumin, an agent for distributing same in water, water and a salt of a sulfonated oil.

8. As a new article of manufacture, a 50 printing color comprising a suitable color and a vehicle containing albumin, an agent for distributing same in water, water, a salt of a sulfonated oil and an ethereal oil.

In testimony, that we claim the foregoing 55 as our invention, we have signed our names in presence of two subscribing witnesses.

LEOPOLD SCHÜTZE.  
ROBERT FISCHER.

Witnesses:

RUDOLPH FRICKE,  
DORIS KRAHL.